

## UNITED STATES PATENT OFFICE

2,371,656

## LUBRICANT COMPOSITIONS

Herschel G. Smith, Wallingford, and Troy L. Cantrell, Lansdowne, Pa., assignors to Gulf Oil Corporation, Pittsburgh, Pa., a corporation of Pennsylvania

No Drawing. Application January 26, 1944,  
Serial No. 519,810

7 Claims. (Cl. 252—51)

This invention relates to improvements in lubricant compositions; and more particularly to light lubricating oil compositions of the type known as household lubricants.

Household lubricants are low viscosity oils intended for lubricating electric fans, guns, and all sorts of light mechanism with exposed surfaces of steel, copper and other metals. In general, such oils are applied and used as a more or less stationary film to protect surfaces exposed to the atmosphere. Plain mineral oils under such conditions do not afford adequate protection against rust or corrosion or both and are open to other objections. Various mineral oil compositions have been proposed, containing substances intended to overcome the limitations of plain mineral oil. None has proved entirely satisfactory. It is difficult to prepare a compounded oil containing a plurality of agents each intended to perform a specific function while not interfering with the others, and many compounded oils show a tendency to discolor or deposit insoluble matter on long standing. This is especially true of fatty oils, particularly castor oil.

One object of the present invention is the provision of a household oil composition which has excellent lubricating properties, which is itself non-corrosive, inert and insensitive to moisture, air, etc., and which has the property of protecting steel and other metal surfaces from rust and other forms of corrosion, even on long exposure to adverse atmospheric conditions; and the provision of such an oil which is clear and light in color as prepared and which even on long standing remains bright and clear without development of haze, sediment or discoloration.

These and other objects are achieved by the provision of a lubricating oil composition, the base of which is a light, highly refined mineral oil of viscosity about 60 to 150 seconds SUV at 100° F.; 100-second oil being especially advantageous. In such an oil are dissolved or blended minor amounts of (1) an amine salt of an organic phosphate, as a rust inhibitor, in amount sufficient to protect steel surfaces from rust when filmed with the composition; (2) an oil-miscible castor oil to serve as an oiliness agent; (3) a refined sperm oil ester or its equivalent as a gum-resistant oiliness agent and stabilizer for the castor oil; and, (4) an oil soluble anti-oxidant.

In preparing our household oil, if desired, each agent can be separately and directly added to the lubricating oil base, but it is more convenient

to blend the several agents together before adding them to the lubricating mineral oil. These particular agents will blend together without mutual deleterious effects, and the resulting composition is readily blended with oils.

1. The rust inhibitor is advantageously an amine salt of isoamyl octyl acid phosphate, prepared by bringing into reaction isoamyl octyl acid phosphate and so-called cocoamine, which is a commercially available material prepared by converting cocoanut oil fatty acids into the corresponding amines. It consists mostly of mono-lauryl amine,  $CH_3(CH_2)_{10}—CH_2—NH_2$ , with minor amounts of adjacent homologues. In preparing the rust inhibitor, the reaction between the amine and the acid phosphate is so controlled as to bring the pH of the product within the range 5.5 to 7.5. This inhibitor is disclosed in our co-pending application, Serial No. 420,438, filed November 25, 1941, and, as disclosed in that application, other amines besides cocoamine can be employed, all belonging to the class of primary fatty amines containing from 8 to 18 carbon atoms. These amines include mono-capryl amine,  $CH_3(CH_2)_6CH_2NH_2$ , mono-lauryl, mono-myristyl, monopalmityl and monostearyl amines. In lieu of this class of inhibitors there can be employed, also with advantage, the reaction product of isoamyl octyl acid phosphate with di-cyclohexyl amine in approximately equimolecular proportions and adjusted to a pH within the range 5.5 to 7.5 as described in our co-pending application, Serial No. 420,439, filed November 25, 1941.

2. As shown in our prior applications, Serial Nos. 420,438 and 420,439, such rust inhibitors are readily soluble in mineral oils and mineral oil solutions thereof, effectively protecting metals against rusting and corrosion when applied thereto. In the present invention we get along with less of this rust inhibitor than would otherwise be necessary by virtue of the presence in our improved composition of ingredients 2 and 3 (see below). These last have some anti-rust properties, but not enough to afford adequate protection were they relied on alone. But their effect, in the proportions indicated, is cumulative with that of the aminophosphate to impart to the composition entirely adequate anti-rust properties.

2. The oiliness agent is, as stated, a mineral oil-miscible castor oil. Castor oil, itself, is not miscible with mineral oils, but it can be processed in known ways to render it oil-miscible. In

general, such modified castor oils are known in the art as miscible castor oils. Certain of the modified castor oils now available are actually soluble in mineral oils. One such type of modified castor oil useful in the practice of the present invention is the partially dehydroxylated castor oil obtained by certain known methods. By partially dehydroxylating the castor oil, it is converted into the modified castor oils which are readily soluble in mineral oils, but which retain the desirable oiliness properties of normal castor oil. This modified castor oil is equally effective as regards steel-to-steel lubrication and lubrication of steel in contact with bronze and other metals. Thus it contributes to the wide range of utility of our oil composition.

While this oil-soluble castor oil is excellent as an oiliness agent, it has a tendency to develop insoluble matters or haze in the course of long standing. We effectively restrain this tendency by incorporation of ingredient no. 3, the monohydric alcohol fatty acid ester.

3. The gum-resistant oiliness agent is advantageously a substantially pure sperm oil ester, free from water and glycerides. This substance was very resistant to oxidation and gumming. Furthermore, in our composition it serves as an excellent solvent or blending agent; it facilitates the preparation of concentrates with the other ingredients, and it prevents development of insoluble matter, haze, sediment, etc. on long standing which might otherwise occur due to the presence of the modified castor oil. Only a small amount of the esters is necessary, sufficient to prevent this last-mentioned effect, in view of the presence of the partially dehydroxylated castor oil which is itself an excellent oiliness agent. In lieu of sperm oil or other fatty mono esters which are essentially oleic acid esters of long chain monohydric alcohols, we can employ similar fatty acid esters of short chain monohydric alcohols: e. g. ethyl oleate, butyl oleate, butyl stearate and ethyl thiolstearate.

4. The fourth ingredient, an oil-soluble anti-oxidant, to retard the formation of oil acids, is a tertiary alkyl phenol anti-oxidant such as that prepared by alkylating a phenol with refinery gas: see U. S. Patent 2,149,759 issued March 7, 1939, to T. L. Cantrell. Examples of this class of material are 2,4,6-tri-tertiary butyl phenol, and 2,6-di-tertiary butyl-para cresol. These oxidation inhibitors are among the few that can be employed in the proportions indicated without developing insoluble matters or darkening in color. They serve as additional stabilizing agents and solvents for the modified castor oil. The mineral oil, itself, is fairly stable, but when there is added an oiliness agent such as partially dehydroxylated castor oil, a compounded oil containing this material will more readily oxidize with development of insoluble matter, if some of this type oxidation inhibitor is not present. Thus in the present invention we add the oil oxidation inhibitor to counterbalance the defects that might otherwise be encountered from the oil-soluble castor oil.

In our prior application, Serial No. 422,008, filed December 6, 1941, we have broadly described such improved oil compositions and household lubricants and methods of preparing the same from the several ingredients set forth ante. As there described, one good example of a composition within the purview of this invention is

compounded with refined lubricating oil of 100 viscosity, SUV, at 100° F., as follows:

|                                                                          | Per cent |
|--------------------------------------------------------------------------|----------|
| Base oil                                                                 | 99.4     |
| Mineral-oil-miscible castor oil                                          | 0.1      |
| Rust inhibitor: di-cyclohexyl amine isoamyl octyl phosphate (pH 5.5-7.5) | 0.1      |
| Sperm oil ester (glycerine-free)                                         | 0.3      |
| 2,4,6-tri-tertiary butyl phenol                                          | 0.1      |

10 The above oil composition exhibits the following properties:

|                         |       |      |
|-------------------------|-------|------|
| Gravity                 | ° API | 28.8 |
| Viscosity, SUV: 100° F. | ° F.  | 103  |
| Flash, OC               | ° F.  | 335  |

|             |      |     |
|-------------|------|-----|
| 15 Fire, OC | ° F. | 375 |
|-------------|------|-----|

Corrosion test (see below):

|                   |      |     |
|-------------------|------|-----|
| Duration of tests | days | 12  |
| Temperature       | ° F. | 122 |

Test strip (see below):

|          |                       |
|----------|-----------------------|
| 20 Steel | Passes (no corrosion) |
| Copper   | Passes (no corrosion) |

|          |         |      |
|----------|---------|------|
| Air rate | cc./hr. | 2000 |
|----------|---------|------|

|              |          |    |
|--------------|----------|----|
| Water added  | per cent | 10 |
| Salt (3.39%) |          |    |

25 In determining the protective properties of our improved oil compositions ante, a drastic test was employed which comprises immersing a steel strip in 36 cc. of oil in a test tube and adding thereto 4 cc. of sea water placing the assembled

30 tube in a water bath controlled at 122° F. and passing 2000 cc. of moist air per hour into the tube at a point near the bottom to mix the oil and water. This test is conducted for 12 days and make-up water is added each 24 hours to 35 maintain the level of water.

In the example ante, the steel test strip in the presence of uncompounded base oil showed rust within 6 hours, whereas the steel strip in the compounded product showed no rust within 12 days. Tests with strips of other metals, e. g. copper, gave similar good results.

40 In the above example, the proportions of the additive agents incorporated in the mineral oil may be varied, if desired as shown in our prior application, Serial No. 422,008.

In general, as disclosed in our Serial No. 422,008, the optimum ranges of proportions for the several constituents are as follows:

|                              | Per cent      |
|------------------------------|---------------|
| Base oil                     | 96.5 to 99.75 |
| Rust inhibitor               | 0.05 to 1.0   |
| Oil-miscible castor oil      | 0.05 to 1.0   |
| Gum-resistant oiliness agent | 0.10 to 1.0   |
| Oil-soluble anti-oxidant     | 0.05 to 0.5   |

55 As there shown, such improved lubricants have many advantageous properties and are particularly useful in protecting metals from rust and corrosion as well as effectively lubricating the same.

60 The present application is a continuation-in-part of our prior application, Serial No. 422,008 filed December 6, 1941. In turn, our application, Serial No. 422,008 is a continuation-in-part of our earlier co-pending application, Serial No. 420,439, filed November 25, 1941.

65 In our prior application, Serial No. 420,439, we have also disclosed improved lubricating oil compositions containing, as a rust inhibitor, a substantially neutral reaction product obtained by reacting isoamyl octyl acid phosphate with di-cyclohexyl amine in approximately equimolecular proportions under such conditions that the reaction product or mixture has a pH between 5.5 and 7.5.

The acid phosphate ester employed as one reactant is a di-ester of ortho-phosphoric acid and has the following formula:



This compound is also known as 3-methyl-butyl, 2-ethyl-hexyl ortho-phosphate.

The other reactant, di-cyclohexyl amine is likewise a well-known chemical compound, commercially available as a substantially pure material; though it is not necessary that a "CP" amine be used. One of the commercial grades advantageous for the present purposes has the following properties:

|                     |      |        |
|---------------------|------|--------|
| Boiling point       | ° F. | 493    |
| Melting point       | ° F. | 32     |
| Sp. gr., 77°/77° F. |      | 0.9104 |
| Flash               | ° F. | 212    |
| Fire                | ° F. | 320    |

The reaction between di-cyclohexyl amine and the acid phosphate ester is exothermic and as described in our prior application, Serial No. 420,439, the temperature is controlled by heating or cooling as required in preparing our rust inhibitors from said amine and phosphate ester by the method set forth in that application. Further, as there described, the reaction products so obtained are substantially neutral. They are relatively stable compositions under ordinary conditions. At room temperatures, they are heavy, viscous, oily liquids. They are relatively non-volatile. Further, these rust inhibitors are insoluble in water and very resistant to hydrolysis, being in fact quite water repellent. On the other hand they are moderately soluble in oils, both mineral and fatty oils, the solubility varying somewhat with the particular oil; for instance, light paraffinic oils such as employed in making household lubricants, etc., dissolve approximately 0.50 per cent by weight of these reaction products, forming stable solutions; naphthenic type mineral oils dissolve somewhat larger amounts.

Accordingly the rust inhibitors described in our application, Serial No. 420,439 are advantageous in preparing improved household lubricants, particularly those containing various fatty oils compounded with the mineral oil, as further described in that application.

The following examples illustrate advantageous methods of preparing these rust inhibitors and improved oils and lubricants containing the same:

*Example I.*—In preparing this particular rust inhibitor, the reaction is carried out in an iron kettle equipped with means for heating and cooling and for agitating the mixture. Into the kettle are introduced 181 pounds of commercial di-cyclohexyl amine, and 281 pounds of commercial isoamyl octyl acid phosphate are gradually added with stirring. The reaction is vigorous and quite exothermic and the acid phosphate is added at such a rate as to facilitate maintaining the reaction temperature below 180° F. The mixture may be cooled if required to maintain it below that temperature. The reaction temperature is best maintained between 140 and 180° F. during the larger portion of the reaction. After all of the acid phosphate has been added, the mixture is ordinarily warmed to facilitate completion of the reaction. At this time the reaction mixture usually has a pH of

3 to 4 and the final adjustment and control of the pH value is then effected. In doing so we add 18 pounds of the amine and the mixture is maintained at approximately 165° F. until it has a pH of approximately 7.2.

The rust inhibitor so obtained is a heavy viscous, oily liquid. Similar viscous oily rust inhibitor can be readily obtained having other pH values within the range of 5.5 to 7.5 by controlled adjustment of the pH during the last stage of the reaction.

The product of this example is sufficiently soluble in mineral oils for making the improved oil compositions in this invention. As the amine, from which the above rust inhibitor is prepared, is also soluble in mineral oils, we sometimes prepare the oily rust inhibitor in situ in the mineral oil. In such embodiments of this invention, the di-cyclohexyl amine is first dissolved in the mineral oil and then the acid phosphate ester added, the mixture being stirred and maintained at the desired temperatures until the reaction is complete and the mixture adjusted to the proper pH value, the added mineral oil serving as a diluent, facilitating control of the reaction. The concentrates or oil solutions of neutral reaction products so obtained are useful addition agents to various types of lubricants. The preparation of such concentrates is illustrated in the following example:

*Example II.*—One hundred pounds of light mineral oil having a viscosity of 100 seconds SUV at 100° F. were added to an iron vessel equipped with means for heating and cooling and agitation. The initial temperature of the oil was 80° F. To this oil were added 181 pounds of di-cyclohexyl amine, which was thoroughly mixed with the oil by mechanical agitation and the final temperature of this mixture was 82° F. To the oil-amine mixture 281 pounds of commercial isoamyl octyl acid phosphate were added over a period of two hours, during which time the temperature of the reaction mixture rose to 188° F. After stirring for one hour, the pH of the mixture was 3.7. In order to increase this value to the desired range, nine pounds of di-cyclohexyl amine were added to the mixture and stirred, and the resultant mixture had a pH of 6.2. To secure a final adjustment, nine additional pounds of di-cyclohexyl amine were added to the mixture which after stirring for one hour and cooling to room temperature, exhibited a pH of 7.4.

The oily mixture prepared in this Example II can be regarded as a sort of concentrated stock solution, which can be stored indefinitely and incorporated in lubricating oils as desired to prepare commercial anti-rust oils, etc.

*Example III.*—A household-type lubricating oil was prepared by dissolving 0.05 per cent by weight of di-cyclohexyl amine isoamyl octyl phosphate, prepared as in Example I. Properties of the new oil and the base oil are tabulated below:

|                          | Inhibited oil | Base oil |
|--------------------------|---------------|----------|
| 65 Gravity, ° A. P. I.   | 28.9          | 28.9     |
| Viscosity, S. U. V.:     |               |          |
| 100° F.                  | 101.4         | 100.7    |
| 210° F.                  | 38.7          | 38.6     |
| Flash, O C. ° F.         | 335           | 335      |
| Fire, O C. ° F.          | 380           | 385      |
| Pour, ° F.               | 40            | 45       |
| Color, N. P. A.          | 1.25          | 1.25     |
| Carbon residue, per cent | 0.02          | Trace    |
| Neutralization No.       | 0.06          | 0.03     |
| Corrosion test:          |               |          |
| Steel strip              | Passes        | Fails    |
| Copper strip             | Passes        | Fails    |

It is sometimes desirable to incorporate oiliness agents and extreme pressure agents in rust-preventive oils; agents such as sperm oil and castor oil which have been processed to render them miscible with mineral oils. According to the present invention, a concentrate can be prepared, including the new rust inhibitor together with oiliness agents, which concentrate can be added to a plain mineral oil in quantity sufficient to impart the required rust preventive and oiliness properties.

*Example IV.*—In preparing such a concentrate, materials are blended together in a suitable vessel in proportions as follows:

| Materials                       | Pounds |
|---------------------------------|--------|
| Sperm oil                       | 60     |
| Oil-soluble castor oil          | 20     |
| Reaction product from Example I | 20     |
| 2,4,6-tri-tertiary butyl phenol | 20     |

The oil-soluble castor oil used in this example was a partially dehydroxylated castor oil which is readily soluble in mineral oils and is available as a commercial material. Likewise, the sperm oil employed was a commercial oil substantially free of glycerides. The properties of the commercial sperm oil and oil-soluble castor oil were as follows:

|                                  | Oil-soluble castor oil | Sperm oil           |
|----------------------------------|------------------------|---------------------|
| Gravity, °A. P. I.               | 16.7                   |                     |
| Sp. gr. 60°/60° F.               | 0.9548                 | 0.878-0.884         |
| Viscosity, S. U. V.:             |                        |                     |
| 100° F.                          | 1,328                  | 95-110.             |
| 210° F.                          | 142.9                  |                     |
| Flash, OC, ° F.                  | 485                    | Min. 400            |
| Fire, OC, ° F.                   | 600                    |                     |
| Pour, ° F.                       | —35                    | Max. 60             |
| Color, N. P. A.                  | 2.25                   | Not darker than 3.0 |
| Carbon residue, per cent.        | 0.48                   |                     |
| Neutralization No.               | 3.20                   | Max. 2.0.           |
| Oleic acid equivalent, per cent. |                        | Max. 1.0.           |
| Iodine No. (modified Hanus).     | 103.8                  | 75-90               |
| Saponification No.               | 190.4                  | 120-140             |

In blending these oils with the rust inhibitor and antioxidant, the procedure was as follows:

The sperm oil was introduced into the kettle and the oil-soluble castor oil gradually added with stirring. The mixture was maintained at a temperature between 60° and 70° F. and the agitation continued until a clear blended oil was obtained. To the blended oil, while continuing the agitation, were added the reaction products from Example I which rust inhibitor readily dissolved in the blended oil. Then the 2,4,6-tri-tertiary butyl phenol was added with agitation and the temperature was brought to 160° F. and held at that temperature until a homogeneous blend was obtained. The warm mixture was then passed through a filter press to remove any traces of insoluble matter. The filtrate so obtained was a clear oily fluid which can be stored indefinitely. It is readily soluble in oil and requires no special blending procedure to incorporate it in mineral lubricating oils in making our improved lubricants. The preparation of one such improved lubricant is illustrated in the following example:

*Example V.*—An improved household oil was prepared by dissolving the composition of Example IV in a light, highly-refined paraffinic mineral oil in such proportions that the improved mineral oil contained 0.1% of the new rust inhibitor, 0.3% of sperm oil, 0.1% of oil-soluble

castor oil and 0.1% to 2,4,6-tri-tertiary butyl phenol.

The properties of the improved household oil as compared with those of the mineral oil alone are tabulated below:

|                                                           | Inhibited oil | Uninhibited base oil |
|-----------------------------------------------------------|---------------|----------------------|
| Physical properties:                                      |               |                      |
| Gravity, °API                                             | 33.5          | 33.5                 |
| Viscosity, S.U.V.:                                        |               |                      |
| 100° F.                                                   | 104.9         | 105.6                |
| 210° F.                                                   | 39.7          | 40.0                 |
| Flash, OC, ° F.                                           | 375.          | 370                  |
| Fire, OC, ° F.                                            | 430           | 430                  |
| Pour, ° F.                                                | 0             | 0                    |
| Color, Saybolt                                            | +13           | +16                  |
| Carbon residue, percent                                   | 0.01          | 0.01                 |
| Neutralization No.                                        | 0.20          | 0.02                 |
| Tests:                                                    |               |                      |
| Corrosion test—                                           |               |                      |
| Steel strip...                                            | Passes...     | Fails...             |
| Copper strip...                                           | do...         | Do.                  |
| Evaporation loss, copper dish, percent:                   |               |                      |
| 212° F., 5 g., 48 hr.                                     |               |                      |
| Appearance of cup...                                      | Fair...       | Good...              |
| Sludge...                                                 | Nil...        | Nil.                 |
| Falex wear test:                                          |               |                      |
| 500 lb. jaw load, 15 min. wear: No. of teeth <sup>1</sup> |               |                      |
| 14                                                        |               | Fails.               |
| Slight oxidation No.                                      | 8             | 5                    |
| Oxidation test: S. H. Kress Co.—                          |               |                      |
| Copper strip test, appearance                             | Medium stain. | Light stain.         |
| Oxidized oil—                                             |               |                      |
| Color, N.P.A.                                             | 5.0           | 1.0                  |
| Neutralization No.                                        | 0.20          | 0.01                 |
| Sludge, percent                                           | Nil           | Nil                  |

<sup>1</sup> One tooth wear is equivalent to 0.0000218" wear on the test shaft and block.

In the above example, the steel test strip in the presence of the un compounded base oil showed rust within 6 hours, whereas the steel strip in the un compounded lubricant showed no rust in 12 days. Tests with strips of other metals, e. g. copper, gave similar good results.

The oiliness properties were evaluated with the aid of a Falex tester, a device making use of a shaft rotated between two well-machined test pieces to which controlled pressure may be applied. Measurement of the wear was made at the end of the test. The improved oil shown in the example in this test developed a wear of only 14 teeth, whereas un compounded oil failed to carry the test load. In order to evaluate the anti-gumming properties, 5 grams of oil were heated in a copper dish at 212° F. for 48 hours and the sludge and gum deposits inspected. Our improved oil showed no evidence of gumming or sludge deposits.

The foregoing specific examples are merely illustrative of certain advantageous embodiments of this invention, and various other commercial embodiments may be employed in the generic practice thereof. For instance, in preparing concentrates or blends of the several agents, as illustrated in Example IV ante, we sometimes employ, in lieu of the reaction products produced in Example I, the concentrated solutions thereof in mineral oil such as produced in Example II; the concentrated solutions of rust inhibitor in mineral oil being completely miscible with the sperm oil and other agents set forth in Example IV. The blended oil compositions so obtained can be incorporated in a wide variety of lubricating oils to improve their rust preventive and lubricating properties. These blends or composite improvement agents comprising a blend of mineral oil, rust inhibitor, oiliness and anti-oxidant agents are useful and advantageous in preparing improved household oiliness and

other commercial lubricants. In general, a wide variety of improved lubricating oils and compositions can be prepared in accordance with this invention as described and illustrated ante.

What we claim is:

1. An improved petroleum oil composition, effective as a lubricant for ferrous and non-ferrous metal surfaces and capable of preventing rusting and corrosion thereof in the presence of moisture and air, comprising a mineral lubricating oil containing 0.05 to 1.0% of a partially dehydroxylated castor oil, 0.10 to 1.0 per cent of a fatty monoester, 0.05 to 0.5 per cent of a tertiary alkyl phenol, and 0.05 to 1.0 per cent of a substantially neutral addition product of 3-methyl-butyl, 2-ethyl-hexyl acid phosphate and di-cyclohexyl amine, dissolved therein, said substantially neutral product containing the said acid phosphate and amine chemically combined together in molar ratios between 1:1 and 1:1.1 and having a pH between 5.5 and 7.5 and being capable of inhibiting the corrosion of said metals in the presence of air and moisture, said partially dehydroxylated castor oil being readily soluble in the mineral oil, but having a tendency to oxidize and develop insoluble matter, said alkyl phenol being 2,4,6-alkyl phenol containing at least one tertiary butyl group and being capable of inhibiting the oxidation of the partially dehydroxylated castor oil, the said fatty monoester being an ester of a fatty acid and a monohydric alcohol and being capable of preventing development of insoluble matter in said composition, all of the said agents being mutually soluble and miscible in the proportions specified and the so-blended composition being a stable, clear, homogeneous solution of said agents in the mineral oil, the said oil solution thereof having excellent oiliness and other lubricating properties on both ferrous and non-ferrous metals, being non-corrosive to such metals, being inert and insensitive to moisture and air, and being free from haze and insoluble matters and stable against discoloration, development of haze, and deposition of insoluble matters.

2. The improved composition of claim 1 wherein said fatty monoester is sperm oil.
3. The improved composition of claim 1 wherein said fatty monoester is butyl oleate.
5. 4. The improved composition of claim 1 wherein said fatty monoester is butyl stearate.
5. The improved composition of claim 1 wherein said tertiary alkyl phenol is 2,4,6-tri-tertiary butyl phenol.
10. 6. The improved composition of claim 1 wherein said tertiary alkyl phenol is 2,6-di-tertiary-butyl paracresol.
7. An improved petroleum oil composition, effective as a lubricant for ferrous and non-ferrous metal surfaces and capable of preventing rusting and corrosion thereof in the presence of moisture and air, comprising a mineral lubricating oil containing 0.1 per cent of a partially dehydroxylated castor oil, 0.3 per cent of sperm oil, 0.1 per cent of 2,4,6-tri-tertiary butyl phenol addition product of di-cyclohexyl amine and 3-methyl-butyl, 2-ethyl-hexyl acid phosphate, dissolved therein, said substantially neutral product containing the said acid phosphate and amine chemically combined together in molar ratios between 1:1 and 1:1.1 and having a pH between 5.5 and 7.5 and being capable of inhibiting the corrosion of said metals in the presence of air and moisture, said partially dehydroxylated castor oil being readily soluble in the mineral oil but having a tendency to oxidize and develop insoluble matter, said 2,4,6-tri-tertiary butyl phenol being capable of inhibiting the oxidation of the partially dehydroxylated castor oil, the sperm oil being capable of preventing the development of insoluble matter in said composition, all of said agents being mutually soluble and miscible in the proportions specified and the so-blended composition being a stable, clear, homogeneous solution of said agents in the mineral oil.

HERSCHEL G. SMITH.  
TROY L. CANTRELL.